

## UNITED STATES PATENT OFFICE.

CHARLES B. JACOBS, OF WILMINGTON, DELAWARE, ASSIGNOR, BY MESNE ASSIGNMENTS, TO ELECTRO METALLURGICAL COMPANY, A CORPORATION OF WEST VIRGINIA.

## CASTING HAVING CHROMIUM ALLOY SURFACE.

No Drawing.

Application filed April 22, 1921. Serial No. 463,565.

This invention relates to ferrous metal castings the surface portions of which are alloyed with chromium, and it comprises, as a new process, the forming of an alloy surface on the casting during the casting operation, and, as a new article of manufacture, a ferrous metal casting, such as cast iron and cast steel, the surface portion of which is alloyed with chromium to such an extent as to substantially increase the resistance of said surface portion to oxidation at high temperatures.

Recent activity in the heat treatment of steel for various purposes has led to a demand for containers which would withstand oxidation of furnace gases at high temperatures. To meet this need certain alloys composed of nickel, chromium and iron, have been devised. These were put on the market under the name of nichrome, pyroloy, nichroloy, hardite, etc. These alloys are all very similar and usually contain from 10-15% chromium, 40-50% nickel, and the balance iron with the usual small constituents of manganese, silicon, carbon, etc., found in iron and steel. Alloys of the above composition are for the most part made by melting up various constituents in the proper proportions in electric furnaces and casting the melt in the shape of heat treating boxes, retorts, muffles, etc. Alloys of this nature are expensive and have been somewhat unreliable on account of the lack of control in the manufacture.

My experience in the construction of cyanide retorts, designed to withstand the action of oxygen-containing gases at a temperature of 2000-2300° F., has led me to believe that such alloys are unsatisfactory on account of the variation in the product obtainable on the market and the high cost of the alloys. One sample of one of the above-named alloys, for example, would resist oxidation almost completely at the above temperature, while the next sample of supposedly the same composition would break down and oxidize badly in a very short time.

Knowing that metallic chromium was resistant to oxidation to an extreme degree even at very high temperatures, it occurred to me that if wrought iron or steel, both of which were cheaper and mechanically stronger than the nickel-chromium alloys

and otherwise better suited to the construction of retorts, could be surfaced with chromium, it would render the steel or iron sufficiently resistant at high temperatures to serve my purpose. The first attempt to accomplish this was by electrolytic deposition of chromium, but this procedure, while working very well on small surfaces, was found impracticable of application to large retorts.

Upon further investigation I have discovered that a casting having a surface portion, or layer, high in chromium can be produced by bringing the casting metal into contact with chromium during the casting operation in a manner which I shall describe hereinafter in detail. By my new procedure, it is possible to produce a chromium alloy coating on a steel casting the thickness of which coating may vary from  $\frac{1}{16}$ " or less to  $\frac{1}{8}$ "- $\frac{1}{4}$ " as desired. This coating in all cases remains on the surface of the casting as a distinct separate layer. It is not impaired in quality by diffusion into the steel casting, even after long service at high temperatures. The coating is firmly fused to the casting itself and cannot be scaled or chipped off, even with the use of an air chisel.

Generally speaking, my new method comprises coating those surfaces of the mold or cores of the mold in which the casting is made, corresponding with the surfaces of the casting on which the alloy is required, with the chromium in a granular condition in such a manner that the casting metal on flowing into the mold permeates and melts or dissolves the metallic coating. The "skin-chill" or chilling effect exerted by the mold surfaces prevents the chromium from diffusing throughout the body of the casting metal so that an alloy is formed on the surface of the casting containing a high percentage of chromium.

To prevent the coating from being washed from the mold surfaces by the flow of the casting metal, the chromium in a granular or comminuted condition is mixed with a suitable binder into a plastic mass and applied to the mold or core surfaces and then dried so that it adheres firmly to the surfaces, forming a more or less porous coating containing spaces between chromium gran-

ules into which the casting metal enters and displaces the binder and melts or dissolves the metallic particles.

It is important to apply the chromium-containing coating evenly all over the mold or the core surfaces, as the case may be, and to have the chromium particles of such size or in such physical condition that spaces between the particles are formed, into which spaces the cast metal can force its way, displacing any flux or binder contained therein and surrounding the particles, and either melt them or take them into solution during the time the casting metal remains in a molten condition in the mold. For this reason it is necessary to size the coating material so that the voids between the particles will be sufficiently large to permit the proper quantity of the particular casting metal to enter the voids and melt or dissolve the chromium.

The new method may be advantageously practiced with chromium particles having a size between 18 and 30 mesh, that is, all of the particles passing through an 18 mesh screen and substantially all of the particles being caught on a 30 mesh screen.

Steel on account of its freedom from the relatively large amount of impurities which go to make up cast iron takes chromium into solution more readily than does cast iron, and offers less difficulty in the formation of alloys on its surface, and on account of the greater purity of the metal the alloy is usually of a superior quality.

For a casting designed for resistance to oxidation at high temperature chromium offers the best metal with which to form the alloy on the casting. Iron and chromium alloys containing as little as 12% of chromium are quite resistant to oxidation at temperatures up to 1400-1600° F. When, however, the temperature reaches 1800 to 2000° F. or above, it requires a considerably larger proportion of chromium on the surface of the alloy to render it resistant to oxidation.

A very thin film of pure chromium on the surface of iron or steel serves to render it resistant to oxidation at extremely high temperatures. Even so thin a film of chromium as may be deposited electrolytically on iron or steel renders it remarkably resistant to oxidation at high temperatures, providing the coating or skin is non-porous and continuous.

My invention may be illustrated in detail by the following example:—

A mold for steel casting is prepared in the ordinary way and the surface of this mold while in the green state, i. e., before baking it (as is usual with molds for steel castings) is coated to the proper depth, for example, to 1/8 of an inch, with comminuted or granulated chromium mixed with ordinary silicate of soda solution. Sufficient

solution is added to the chromium to form a plastic mass which can be applied with a molding tool evenly all over the mold or core surface it is desired to coat. With a mixture of the right consistency, each square foot of coating 1/8" thick will contain about 1.2 lbs. of chromium. The silicate of soda causes the chromium to adhere to the surface of the sand composing the mold and after baking the mold to a temperature of about 600-700° F. (i. e. the usual temperature of baking molds for steel castings) the metallic chromium is cemented to the surface of the mold so firmly that it can be rubbed or brushed with the hand without dislodging it. After the mold has been so prepared the casting of the metal is carried out in the usual manner. A pouring temperature of approximately 2650-2900° F. is usually found to be suitable for castings, the molds of which are coated with chromium to the depth of as much as 1/4". If the chromium is comminuted to too fine a state of division, for instance, finer than 50 mesh, and the molten steel has a temperature of about 2650-2700° C., the voids between the metallic particles in the coating are too small to permit a sufficient quantity of the steel to enter them and remain molten long enough to dissolve and take the particles of chromium into solution in the steel. When such is the case only a very thin alloy of chromium will be produced on the surface of the casting which under the microscope will reveal the fact that a part at least of the chromium grains are merely embedded in a matrix of steel and have not lost their identity as shown by their original crystalline structure and traces of original contour. Also the casting is apt to show spots in which little or no chromium has been taken up by the steel.

Silicate of soda gives the best results as a binder although other binders such as "glutrin" (a commercial product obtained by concentrating sulphite waste liquor), molasses or similar tacky substances may be used for causing the chromium to adhere to the surface of the mold, but irrespective of the particular binder used, only a sufficient quantity to just accomplish firm adherence of the coating to the mold should be used. An excess of binder destroys porosity of the coating and is difficult to displace by the casting metal.

It will be noted in the above example that although the temperature at which the metal is poured in forming a chromium alloy on cast steel may be somewhat below the melting point of the chromium, yet, as there is evidence to show, a true alloy is formed on the steel casting and not a mere surface overlay. However, where the chill caused by the mold is excessive a temperature of 2750° F., or more is preferred.

I have in practice made castings with steel on which high chromium alloy penetrating to a depth of  $\frac{1}{8}$ " was obtained on the surface of the casting in a retort weighing 5 276 lbs., and to the depth of  $\frac{1}{4}$ " in a retort weighing 10670 lbs.

As an example of the resistance to oxidation at high temperatures of such castings in actual service may be cited the results 10 obtained under the following conditions with the small retort mentioned above. The retort was put into service and continually operated for 29 days at the end of which period it showed no signs of having been 15 oxidized by the combustion chamber gases of the furnace which contained a large excess of oxygen. The conditions under which the retort was operated were as follows:

Temperature inside the retort 1760-1790° 20 F., temperature of combustion chamber gases in contact with outside of retort 2112-2200° F., duration of the heating 29 days, weight of retort at end of test 278 lbs., weight of retort before test 276 lbs., 25 increase in weight by oxidation 2 lbs. or 7.2%.

At the same time this test was made a solid cylinder of steel 2" in diameter and 30" long poured from the same ladle of 30 metal used in pouring the retort but unprotected by chromium was placed in the furnace with the retort and left there during the entire test. The unprotected cylinder was oxidized to a depth of from  $\frac{1}{2}$  to 1" 35 and very badly distorted and swollen beyond its original diameter. It contained only a core of unoxidized metal in the center.

Sections cut from the retort and samples 40 for analysis taken by machine cuttings and drillings throw considerable light on what took place during the casting operation. Since the steel was poured into the mold at a temperature (2650° F.) below the melting point (2741° F.) of the 98 to 99% 45 chromium with which the mold was surfaced, the melted steel coming in contact with the chromium dissolved some of the chromium from the coating. This lowered 50 the melting point of the steel and kept it molten until all of the chromium coating was dissolved. The "skin-chill" of the mold surfaces exerted a chilling effect before complete diffusion of the chromium could take 55 place and the freezing of the alloy, starting at the mold surfaces, took place so rapidly that as a consequence an alloy high in chromium, containing 39.56% chromium in the first  $1/100$  of an inch next to the mold 60 surface and grading off to 9.45% at a depth of  $\frac{1}{8}$  of an inch below the surface, was built up on the surface of the casting. That 65 this is a true alloy and not a mere coating or overlay of melted chromium fused into the surface of the steel is shown by the

chromium content at different depths in the section of the casting given in the following table:

| Location of sample.                              | Per cent chromium. | 70 |
|--------------------------------------------------|--------------------|----|
| 1. Skin to depth of $1/100$ " (machine cuttings) | 39.56              |    |
| 2. Additional $1/100$ " (machine cuttings)       | 38.51              |    |
| 3. Skin to depth of $1/16$ " (machine cuttings)  | 31.08              |    |
| 4. Skin to depth of $1/8$ " (drilling)           | 9.45               |    |
| 5. $1/2$ " from face of casting (drilling)       | 0.86               | 75 |
| 6. $1$ " from face of casting (drilling)         | 0.37               |    |

The steel which was used for the casting on which the above tests were made contained 0.00% of chromium. The analysis 80 of the heat from which this casting was poured is as follows:

|            | Per cent. | 80 |
|------------|-----------|----|
| Carbon     | 0.28      |    |
| Manganese  | 0.65      | 85 |
| Silicon    | 0.282     |    |
| Phosphorus | 0.039     |    |
| Sulphur    | 0.041     |    |

Cast steel retorts with a high chromium alloy on the surface similar in composition to that just shown above have proved more resistant to oxidation at high temperatures, under the same conditions, than iron-chromium-nickel alloys containing from 50 to 65% of nickel and 10 to 20% of chromium. In addition to greater resistance to oxidation, cast steel with a high chromium alloy on the surface possesses the strength and soundness inherent in steel castings.

Although cast iron is less desirable than steel for apparatus which is to be used at high temperatures, it may be expedient in some cases to use cast iron to form the body of the casting which is to be provided with a chromium alloy surface. It becomes necessary in this case to modify the procedure described above in connection with steel to the extent that the cast iron should be at a higher temperature when poured than is necessary with steel, since the impurities existing in cast iron which total about 8 to 10% tend to prevent the chromium from going into solution in the cast iron, unless the latter be raised to a high temperature, say slightly above 2741° F., the melting point of chromium. This offers no serious difficulty since by the use of thermit the iron in the ladle may be easily raised to a temperature of 2800 to 2900° F. before pouring it into the molds.

Instead of substantially pure chromium as the substance to be alloyed with the cast iron or steel, I may use a ferro-chrome containing a high percentage of chromium. The pure chromium is preferred, however, on account of the higher chromium content obtainable on the face of the casting.

An iron or steel casting obtainable by my new method and having as an integral part thereof an iron-chromium alloy surface con-

taining more than 20% of chromium while the major portion of the casting contains less than 15% of chromium, is, as far as I know, a new article of manufacture.

5. Various changes in minor details may be made in the method above described without departing from the spirit and scope of my invention.

I claim:—

10. 1. The method of making a ferrous metal casting having a chromium alloy surface layer that is strongly resistant to oxidation, which comprises coating a surface in the mold in which the casting is to be formed to a depth of from about one-eighth to one-quarter of an inch with a mixture composed of metallic particles comprising chromium and a binder for said particles, hardening the resulting coating, and then introducing into said mold molten ferrous metal at a pouring temperature of from about 2650 to 2900° F., the size and disposition of said metallic particles in the coating being such as to permit ready penetration therebetween by the 25 molten metal and solution of said particles by said molten metal.

2. The method of making a ferrous metal casting having a chromium alloy surface layer that is strongly resistant to oxidation at high temperatures, which comprises coating a surface in the mold in which the casting is to be formed to a depth of from about one-eighth to one-quarter of an inch with a mixture comprising a sodium silicate solution and substantially pure chromium comminuted to a size between 18 and 30 mesh, baking the coated mold, and then introducing into the baked mold molten ferrous metal at a pouring temperature of from 40 about 2650 to 2900° F.

3. As a new article of manufacture, a ferrous metal casting alloyed at its surface with chromium, the latter forming a distinct layer in which the chromium content decreases from the surface toward the interior of the ferrous metal and is sufficiently high at the surface to render the casting resistant to oxidation at temperatures up to at least 1800° F.

4. As a new article of manufacture, a ferrous metal casting alloyed at its surface with chromium, the surface layer consisting essentially of chromium and having a chromium content substantially greater than that of the interior of the ferrous metal, the percentage of chromium at the surface being sufficient to render the casting resistant to oxidation at temperatures up to at least 1800° F.

5. As a new article of manufacture, a steel casting alloyed at its surface with chromium, the surface layer for a depth of at least an eighth of an inch containing more than 25% chromium, the chromium content decreasing rapidly from said surface layer to the interior of the casting.

6. As a new article of manufacture, a steel casting alloyed at its surface with chromium, the alloyed portion forming a distinct layer having a thickness of 1/16 to 1/4 of an inch and consisting essentially of chromium at the surface, and in which the chromium content is more than 25% at a depth of 1/16 of an inch and decreases progressively to less than 15% at a depth of 1/8 of an inch.

7. As a new article of manufacture, a steel casting containing chromium in the form of an alloy, the chromium content at the surface of the casting being greater than 25% and at an eighth of an inch below the surface, less than 15%.

8. As a new article of manufacture, a steel casting containing chromium in the form of an alloy, the chromium content of a surface layer 1/100 of an inch in thickness being greater than 38% and at an eighth of an inch below the surface, less than 15%.

9. As a new article of manufacture, a steel casting containing chromium in the form of an alloy, the body of the casting containing on an average less than 10% of chromium, and a surface layer 1/50 of an inch in thickness containing more than 35% of chromium, the chromium content decreasing rapidly from the surface to the interior.

In testimony whereof I affix my signature.

CHARLES B. JACOBS.